

June 10, 1947.

R. B. COLLINS ET AL

2,422,080

PHOTOGRAPHIC EMULSIONS CONTAINING SUPERSENSITIZING DYE COMBINATIONS

Filed Dec. 6, 1944



*Fig. 1*



*Fig. 2*



*Fig. 3*



*Fig. 4*



*Fig. 5*



*Fig. 6*

*Roland Bernard Collins  
Harold Owen Dickinson* INVENTORS

BY

*Lynn Barrett Morris  
ATTORNEY*

UNITED STATES PATENT OFFICE

2,422,080

# PHOTOGRAPHIC EMULSIONS CONTAINING SUPERSENSITIZING DYE COMBINATIONS

Ronald Bernard Collins and Harold Owen Dickinson, Ilford, England, assignors to Ilford Limited, Ilford, England, a British company

Application December 6, 1944, Serial No. 566,822  
In Great Britain December 8, 1943

7 Claims. (Cl. 95—7)

1

This invention relates to photographic materials and particularly to the manufacture of dye-sensitised photographic silver halide emulsions.

Photographic silver halide emulsions have a certain natural sensitivity to light, but this is restricted to a short range of wavelengths in the ultra-violet and/or blue regions of the spectrum. The effect of incorporating a sensitising dye is to impart to the emulsion sensitivity to light of other wavelengths. It has been known for some time that the effect of incorporating two or more sensitising dyes in the emulsion is not always the simple sum of their individual effects, and sometimes an additional sensitivity is obtained. Combinations of dyes which give this latter result are known as supersensitising combinations.

The present invention is concerned with supersensitising combinations of dyestuffs. According to the invention, photographic silver halide emulsions are supersensitised by incorporating in the emulsion a combination of a sensitising dyestuff of the general formula I.



and a sensitizing dyestuff of the general formula II.



where  $R_1$ ,  $R_2$ ,  $R_3$ ,  $R_5$  and  $R_6$  are the same or different and are alkyl or aralkyl groups or substituted groups of this type,  $R_4$  and  $R_7$  are the same or different and are hydrogen atoms or alkyl or aralkyl groups,  $D_1$ ,  $D_2$ ,  $D_3$  and  $D_4$  are the same or different and are residues of heterocyclic nitrogen nuclei of the type common in cyanine dyes, and  $X$  and  $Y$  are the same or different and are acid radicles and  $n$  is 0 or 1.

In cases where the R groups, or any of them, are alkyl radicles, these are preferably lower alkyl radicles, i. e. containing not more than 4 carbon atoms, e. g. methyl, ethyl, or hydroxyethyl radicles, though they may be higher alkyl radicles. In cases where the R groups, or any of them, are aralkyl radicles, they may be, for example, benzyl or naphthylmethyl radicles. Substituted alkyl radicles which may be present, e. g. as any of R<sub>1</sub>, R<sub>2</sub>, R<sub>5</sub> and R<sub>6</sub>, may be hydroxyalkyl radicles.

The residues  $D_1$ ,  $D_2$ ,  $D_3$  and  $D_4$  may be selected from the residues of thiazoles, oxazoles, selenazoles and their polycyclic homologues, such as

those of the benzene, naphthalene, acenaphthene and anthracene series, pyridine and its polycyclic homologues, such as quinoline and  $\alpha$  and  $\beta$  naphthaquinolines, lepidines, indolenines, diazines, such as pyrimidines and quinazolines, diazoles (e. g. thio- $\beta,\beta'$ -diazole), oxazolines, thiazolines and selenazolines. The polycyclic compounds of this series may also be substituted in the carbocyclic rings with one or more groups such as alkyl, aryl, amino, hydroxy, alkoxy and methylene-dioxy groups, or by halogen atoms.

The acid radicles X and Y may be, for example, selected from halogenide radicles, e. g. chloride, bromide and iodide, or alkyl sulphate, alkyl p-toluene sulphonate or perchlorate.

Dyestuffs of the general formula I, and their preparation, are described in British patent specification No. 553,144 and corresponding United States application Serial Number 461,324 filed October 8, 1942. Dyestuffs of the general formula II are well known and may be synthesised by any of the known methods.

The following are examples of specific dyestuffs which may be employed, the dyestuffs being lettered to facilitate subsequent reference:

### *Dyestuffs of general formula I*

- 30 A. 3,3'-di(hydroxyethyl)-9-methyl-thiadicarbocyanine iodide.  
B. 3-ethyl-3',9-dimethyl-thiaselenadicarbocyanine iodide.  
C. 3,3'-diethyl-9-methyl-thiadicarbocyanine iodide.  
D. 3,3'-diethyl-5,5',9-trimethyl-thiadicarbocyanine iodide.  
35 E. 3,9-dimethyl-3'-ethyl-thiadicarbocyanine iodide.  
F. 3,3',9-triethyl-thiadicarbocyanine iodide.  
G. 3,3'-dimethyl-9-ethyl-thiadicarbocyanine iodide.  
40 H. 2,1',9-trimethyl-thiaquinoddicarbocyanine iodide.  
I. 3,3',9,12-tetramethyl-thiadicarbocyanine iodide.

### Dyestuffs of general formula II

- P. 3,3'-diethyl-9-methyl-thiacarbocyanine bromide.  
 Q. 3,3'-triethyl - 5,5' - dichloro-thiacarbocyanine chloride.  
 50 R. 3,3'-diethyl-9-methyl-4,5,4',5'-dibenz-thia-carbocyanine bromide.  
 S. 3,3'-diethyl-thiacarbocyanine iodide.  
 T. 3,3'-di(hydroxyethyl)-9-methyl-thiacarbocyanine iodide.  
 55

U. 3,3'-diethyl-9-methyl-4,5,4',5'-tetroxydimethylene thiacarbocyanine iodide.

V. 3,3'-diethyl-9-methyl-selenacarbocyanine iodide.

W. 3,3'-triethyl-selenacarbocyanine iodide.

The optimum quantity of such dyestuffs incorporated in the emulsion varies with the particular dyestuff involved. In general, however, proportions equivalent to 5 to 50 cc. of a 1 in 2000 solution of the dyestuff per litre of emulsion are suitable. The dyestuffs are preferably incorporated in the emulsion during the manufacture of the emulsion.

The following examples illustrate the invention. In these examples the emulsions containing the dyes were tested for speed to daylight and to "red" light. The dyestuffs of general formula II, when used alone, do not impart any sensitivity to the emulsion at wavelengths above 680 m $\mu$ , so that by exposing the supersensitised emulsion through a filter which cuts off all radiation of wavelengths less than 680 m $\mu$ , the "red" speed of the emulsion may be determined and this, in comparison with an emulsion containing only a dye of general formula I, affords a measure of the supersensitising effect.

#### Examples

In these examples the dyestuffs employed are referred to by the lettering given above.

The combinations of dyestuffs were incorporated in a gelatin silver iodobromide emulsion containing about 6.5 gms. of silver halide (calculated as silver) per litre of emulsion, during the manufacture of the emulsion, and the resulting emulsion was coated on glass and its speed determined to daylight and also to red light, i. e. of wavelengths above 680 m $\mu$ .

The results obtained are set out in the following table (in which the quantities of dyestuff are given as ccs. of a 1 in 2000 solution of the dyestuff added per litre of emulsion):

| Example No. | Dye of Formula I | Quantity of Dye of Formula I | Dye of Formula II | Quantity of dye of Formula II | Daylight Speed | Red Speed |
|-------------|------------------|------------------------------|-------------------|-------------------------------|----------------|-----------|
| 1a          | A                | 30                           | None              |                               | 140            | 20        |
| 1b          | A                | 30                           | P                 | 30                            | 250            | 64        |
| 2           | A                | 30                           | R                 | 15                            | 150            | 32        |
| 3a          | B                | 30                           | None              |                               | 100            | 18        |
| 3b          | B                | 30                           | P                 | 30                            | 200            | 34        |
| 4a          | B                | 30                           | None              |                               | 89             | 14        |
| 4b          | B                | 30                           | R                 | 30                            | 150            | 25        |
| 5a          | E                | 30                           | None              |                               | 140            | 2.1       |
| 5b          | E                | 30                           | P                 | 30                            | 240            | 9.7       |
| 6a          | C                | 15                           | None              |                               | 250            | 42        |
| 6b          | C                | 15                           | P                 | 12                            | 470            | 89        |
| 7a          | C                | 15                           | None              |                               | 74             | 12        |
| 7b          | C                | 15                           | S                 | 30                            | 260            | 45        |
| 8a          | C                | 15                           | None              |                               | 100            | 21        |
| 8b          | C                | 15                           | T                 | 30                            | 270            | 45        |
| 9a          | D                | 15                           | None              |                               | 74             | 2.8       |
| 9b          | D                | 15                           | S                 | 30                            | 170            | 27        |
| 10          | D                | 15                           | P                 | 30                            | 270            | 38        |

The speed values given in the foregoing table are substantially linearly related, i. e. are in direct proportion. Thus, in the case of Example 3, the daylight speed of the emulsion containing both types of dye (Example 3b) is double that of the same emulsion containing only a dyestuff of the general formula I (Example 3a).

It will be apparent from the data given in the foregoing table that the supersensitising combinations of dyestuffs of this invention in many cases not only impart an increased sensitivity to the emulsion in the sensitising region of the dicarbocyanine dye, but actually effect an increase in the overall sensitivity of the emul-

sion as shown by the generally increased daylight speed.

This general effect is illustrated in the accompanying drawings which show spectral sensitivity curves for the emulsions of certain of the foregoing examples.

In these drawings, Fig. 1 shows the spectral sensitivity curve of the emulsion of Example 1a (full line) and 1b (dotted line), Fig. 2 shows the spectral sensitivity curve of the emulsion of Example 6a (full line) and 6b (dotted line), Fig. 3 shows the spectral sensitivity curve of the emulsion of Example 9a (full line) and 9b (dotted line), Fig. 4 shows the spectral sensitivity curve of the emulsion of Example 3a (full line) and 3b (dotted line), Fig. 5 shows the spectral sensitivity curve of the emulsion of Example 4a (full line) and 4b (dotted line), and Fig. 6 shows the spectral sensitivity curve of the emulsion of Example 5a (full line) and 5b (dotted line).

The dyes of general formula II used in the foregoing examples do not, when used alone, impart any sensitivity to the emulsion over wavelengths longer than 680 m $\mu$  so that the curves clearly demonstrate the supersensitising effect obtained.

While this invention is of particular value in connection with the supersensitising of silver halide emulsions in gelatin, other binding colloids for the emulsion may be employed, for example polyvinyl alcohol, polyvinyl acetals, far-hydrolysed cellulose esters and the like.

What we claim is:

1. A photographic silver halide emulsion containing both a sensitising dyestuff of the formula:



and a sensitising dyestuff of the formula:



where R<sub>1</sub>, R<sub>2</sub>, R<sub>3</sub>, R<sub>5</sub> and R<sub>6</sub> are each selected from the group consisting of alkyl and aralkyl groups, R<sub>4</sub> and R<sub>7</sub> are each selected from the group consisting of the hydrogen atom and alkyl and aralkyl groups, D<sub>1</sub>, D<sub>2</sub>, D<sub>3</sub> and D<sub>4</sub> are residues of heterocyclic nitrogen nuclei of the type common in cyanine dyes, and X and Y are acid radicles and n is a number taken from the group consisting of 0 and 1.

2. A photographic silver halide emulsion containing both a sensitising dyestuff of the formula:



and a sensitising dyestuff of the formula:



where R<sub>1</sub>, R<sub>2</sub>, R<sub>3</sub>, R<sub>5</sub> and R<sub>6</sub> are each selected from the group consisting of alkyl and aralkyl groups, R<sub>4</sub> and R<sub>7</sub> are each selected from the group consisting of the hydrogen atom and alkyl and aralkyl groups, D<sub>1</sub>, D<sub>2</sub>, D<sub>3</sub> and D<sub>4</sub> are residues of azole nuclei, and X and Y are acid radicles and n is a number taken from the group consisting of 0 and 1.

5

3. A photographic silver halide emulsion containing both a sensitising dyestuff of the formula:



and a sensitising dyestuff of the formula:



where  $R_1$ ,  $R_2$ ,  $R_3$ ,  $R_5$  and  $R_6$  are each selected from the group consisting of alkyl and aralkyl groups,  $R_4$  and  $R_7$  are each selected from the group consisting of the hydrogen atom and alkyl and aralkyl groups,  $Z_1$ ,  $Z_2$ ,  $Z_3$  and  $Z_4$  are selected from the group consisting of oxygen, sulphur and selenium atoms, and  $M_1$ ,  $M_2$ ,  $M_3$  and  $M_4$  are residues completing azole nuclei.

4. A photographic silver halide emulsion containing both a sensitising dyestuff of the formula:



and a sensitising dyestuff of the formula:



where  $R_1$ ,  $R_2$ ,  $R_3$ ,  $R_5$  and  $R_6$  are each selected from the group consisting of alkyl and aralkyl groups,  $R_4$  and  $R_7$  are each selected from the group consisting of the hydrogen atom and alkyl and aralkyl groups,  $Z_1$ ,  $Z_2$ ,  $Z_3$  and  $Z_4$  are selected from the group consisting of oxygen, sulphur and selenium atoms, and  $M_1$ ,  $M_2$ ,  $M_3$  and  $M_4$  are residues completing azole nuclei carrying a fused benzene ring.

5. A photographic silver halide emulsion containing both a sensitising dye of the formula:



and a sensitising dye of the formula:



6

where  $R_1$ ,  $R_2$ ,  $R_3$ ,  $R_5$  and  $R_6$  are each lower alkyl groups,  $R_4$  and  $R_7$  are selected from the group consisting of hydrogen and alkyl and aralkyl groups, and  $Z_1$ ,  $Z_2$ ,  $Z_3$  and  $Z_4$  are each selected from the group consisting of oxygen, sulphur and selenium atoms.

6. A photographic silver halide emulsion containing both a sensitising dye of the formula:



and a sensitising dye of the formula:



25 where  $R_1$ ,  $R_2$ ,  $R_3$ ,  $R_5$  and  $R_6$  are lower alkyl groups, and  $R_4$  and  $R_7$  are selected from the group consisting of hydrogen and alkyl and aralkyl groups.

7. A photographic silver halide emulsion containing both a sensitising dye of the formula:



and a sensitising dye of the formula:



where  $R_1$ ,  $R_2$ ,  $R_3$ ,  $R_5$  and  $R_6$  are lower alkyl groups, and  $R_7$  is selected from the group consisting of hydrogen and alkyl and aralkyl groups.

RONALD BERNARD COLLINS.  
HAROLD OWEN DICKINSON.

#### REFERENCES CITED

55 The following references are of record in the file of this patent:

#### UNITED STATES PATENTS

| Number       | Name | Date          |
|--------------|------|---------------|
| 60 2,075,048 | Mees | Mar. 30, 1937 |
| 2,104,064    | Zeh  | Jan. 4, 1938  |